

## UNITED STATES PATENT OFFICE

THEODOR KIRCHEISEN, OF DESSAU IN ANHALT, AND JOHANNES GUERTLER, OF OFFENBACH-ON-THE-MAIN, GERMANY, ASSIGNEES TO GENERAL ANILINE WORKS, INC., OF NEW YORK, N. Y., A CORPORATION OF DELAWARE

## PROCESS OF PRODUCING FAST DYEINGS ON THE FIBER

No Drawing. Original application filed January 21, 1927, Serial No. 162,673, and in Germany January 23, 1926. Divided and this application filed January 18, 1928. Serial No. 247,745.

A known method of producing fast dyeings on the fiber consists in impregnating the fiber with a compound adapted to be coupled and then treating the fiber with a solution of a diazo compound. In cases in which the compound adapted to be coupled has a certain affinity for the fiber it is sufficient merely to wring out the impregnated fiber and to conduct the coupling without previously drying. In producing printed colors, the material is previously prepared with a compound adapted to be coupled, such as for example 2-hydroxynaphthalene, and is printed with a thickened diazo-solution; or the material may be printed with a mixture of an alkali compound of a 2-hydroxynaphthalene carboxylic acid arylamide and a stable diazo compound, after which the material is steamed or exposed to the air and the dyeing developed by treatment with an acid.

In the known process, difficulties are associated with the diazotization. By the present invention these difficulties are avoided and the process is conducted very simply by carrying out the preparation of the diazo compound on the fiber where it unites directly with the coupling component. The preliminary preparation of a diazo-solution or the use of a stable diazo compound is accordingly unnecessary.

In the copending application Serial Number 62,149 filed October 12, 1925, there are described preferred procedures for the preparation of a diazo compound on the fiber and its combination with a coupling component present on the fiber. We do not claim what is disclosed and claimed in the mentioned application but only an improvement of said invention.

According to the present improvement which is a division of Serial No. 162,673 filed January 21, 1927, the invention may be carried out as follows:

The fiber is treated with a mixture of a compound adapted to be coupled and a nitrite and then, after drying, with a solution containing a salt of a diazotizable base, preferably with an addition of an organic acid. One of the treatments with chemicals may be executed by printing.

The following examples, without limiting the invention, serve to illustrate in which manner the process may be carried out:

*Example 1.*—3 grams of di-acetoacetic acid-ortho-tolidinide, 3 cc. of Turkey red oil, 4.5 cc. of sodium hydroxide solution of 34° Bé. and 2 grams of sodium nitrite are dissolved in 40 cc. of water. After addition of 40 grams of neutral starch-tragacanth thickening (6:100) the mixture is printed on unprepared goods. After drying there follows at the ordinary temperature a treatment with a solution of 5 grams of 2-chloro-1-amino-benzene hydrochloride and 20 grams of aluminum sulfate per liter. The goods are washed and soaped hot. There is obtained a clear yellow.

*Example 2.*—There are mixed together solutions of 5 grams of the sodium salt of the acid sulfuric acid ester of leuco-indigo in 20 cc. of water and 5 grams of di-acetoacetic acid-orthotolidinide, 5 cc. of Turkey red oil, 7.5 cc. of sodium hydroxide solution of 34° Bé. in 20 cc. of water and 4 grams of sodium nitrite in 10 cc. of water; to these solutions 50 grams of neutral starch-tragacanth thickening (6:100) are admixed. The unprepared goods are printed with the mixture, dried and then treated with a boiling hot solution containing per liter 0.95 gram of 2,5-dichloro-1-amino-benzene-hydrochloride, 3 cc. of hydrochloric acid of 20° Bé., 50 grams of sodium chloride and 12.5 grams of aluminum sulfate. After they are washed the goods are soaped hot. There is obtained a green dyeing.

*Example 3.*—1.25 grams of 2-hydroxynaphthalene-3-carboxylic acid phenylamide, 3 cc. of Turkey red oil, 2.2 cc. of sodium hydroxide solution of 34° Bé. and 3.8 grams of sodium nitrite are dissolved in 40 cc. of water. After addition of 40 grams of neutral starch-tragacanth thickening (6:100) the unprepared goods are printed with the mixture. They are then dried and introduced into a boiling hot solution containing per liter 0.95 gram of 2,5-dichloro-1-aminobenzene hydrochloride and 15 grams of aluminum sulfate. They are then washed and hot soaped. There is obtained a reddish orange dyeing.

*Example 4.*—1 gram of 2-hydroxy-naphthalene-3-carboxylic acid-4-methoxyphenylamide, 3 cc. of sodium hydroxide solution of 34° Bé., 1.5 cc. of Turkey red oil and 2 grams of sodium nitrite are dissolved in 40 cc. of water. After addition of 40 grams of neutral starch-tragacanth thickening (6:100) the unprepared goods are printed with this mixture. After they have been dried they are treated with a boiling hot solution of 0.5 gram 1-methyl-2-amino-5-nitrobenzene, 7.5 cc. of acetic acid of 30 per cent strength, 50 grams of sodium chloride and 5 grams aluminium sulfate per liter. After they have been rinsed they are soaped hot. There is obtained a Bordeaux tint.

*Example 5.*—The goods are saturated with a solution containing per liter 5 grams of 2-hydroxynaphthalene-3-carboxylic acid-3'-nitrophenylamide, 7.5 cc. of sodium hydroxide solution of 34° Bé., 10 cc. of Turkey red oil (sodium salt) and 10 grams of sodium nitrite. After drying, the goods are printed with the mixture of 5 grams 1-methoxy-2-amino-5-nitrobenzene hydrochloride, 50 grams of lactic acid of 50 per cent strength, 445 grams of water and 500 grams of neutral starch-tragacanth thickening. They are then dried, washed, soaped hot, washed, first hot and then cold, and finally dried. There is obtained a bluish rose color.

*Example 6.*—The goods are saturated with a solution containing per liter 20 grams of diacetoacetic acid-ortho-tolidinide, 30 cc. of sodium hydroxide solution of 34° Bé., 20 grams of Turkey red oil (sodium salt) and 20 grams of sodium nitrite. They are then dried and printed with a mixture of 16 grams 2-chloro-1-aminobenzene hydrochloride, 50 grams of glycolic acid, 434 grams of water and 500 grams of neutral starch-tragacanth thickening. They are then washed, soaped, further washed and dried. There is obtained a clear greenish yellow dyeing.

*Example 7.*—The goods are saturated with a solution containing per liter 25 grams of 2-hydroxynaphthalene, made into a paste with 25 grams of sodium hydroxide solution of 34° Bé. and 20 grams of Turkey red oil (sodium salt) and dissolved in water, and 30 grams of sodium nitrite. After the goods have been dried they are printed with a mixture of 30 grams of 1-aminonaphthalene hydrochloride, 30 grams of formic acid of 90 per cent strength, 440 grams of water and 500 grams of neutral starch-tragacanth thickening, and are then washed and soaped. There is obtained a deep Bordeaux tint.

*Example 8.*—The goods are saturated with a solution containing per liter 20 grams of 2-hydroxynaphthalene-3-carboxylic acid phenylamide, 30 cc. of sodium hydroxide solution of 34° Bé., 20 cc. of Turkey red oil (sodium salt) and 30 grams of sodium nitrite. After they have been dried the goods are

printed with a mixture of 24 grams of 2-amino-1-methoxybenzene-azo-1-amino-naphthalene (or the corresponding sulfamino acid), 8 grams of hydrochloric acid of 20° Bé., 40 grams of acetin, 24 grams of formic acid of 90 per cent strength, 80 grams of lactic acid of 100 per cent strength, 324 grams of water and 500 grams of neutral starch tragacanth thickening. They are then dried, washed and soaped hot. There is obtained a neutral black.

What we claim is:

1. A process for producing fast dyeings on the fiber which consists in treating the fiber with a mixture containing a compound adapted to be coupled and a nitrite, and then, after drying, with a solution containing a salt of a diazotizable base.

2. A process for producing fast dyeings on the fiber which consists in treating the fiber with a mixture containing a compound adapted to be coupled and a nitrite, and then, after drying, with a solution containing a salt of a diazotizable base and an organic acid.

3. A process for producing fast dyeings on the fiber which consists in treating the fiber with a mixture containing a compound adapted to be coupled and a nitrite, and then, after drying, with a solution containing a salt of a diazotizable base, one of the said treatments of the fiber with chemicals being executed by printing.

4. A process for producing fast dyeings on the fiber which consists in treating the fiber with a mixture containing a compound adapted to be coupled and a nitrite, and then, after drying, with a solution containing a salt of a diazotizable base and an organic acid, one of the said treatments of the fiber with chemicals being executed by printing.

5. A process for producing fast dyeings on the fiber which consists in treating the fiber with a mixture containing a compound adapted to be coupled and a nitrite, and then, after drying, printing on a mixture containing a salt of a diazotizable base.

6. A process for producing fast dyeings on the fiber which consists in treating the fiber with a mixture containing a compound adapted to be coupled and a nitrite, and then, after drying, printing on a mixture containing a salt of a diazotizable base and an organic acid.

In testimony whereof, we affix our signatures.

THEODOR KIRCHEISEN.  
JOHANNES GUERTLER.

120

125

130

CERTIFICATE OF CORRECTION.

Patent No. 1,736,083.

Granted November 19, 1929, to

THEODOR KIRCHEISEN ET AL.

It is hereby certified that error appears in the printed specification of the above numbered patent requiring correction as follows: Page 1, line 83, for the word "and" read "of"; and that the said Letters Patent should be read with this correction therein that the same may conform to the record of the case in the Patent Office.

Signed and sealed this 24th day of December, A. D. 1929.

M. J. Moore,  
(Seal) Acting Commissioner of Patents.